

# United States Patent [19]

[11] 3,926,023

Hayashi et al.

[45] Dec. 16, 1975

[54] HYDROSTATIC EXTRUSION PROCESS FOR PRODUCING FINE GAUGE WIRES

[75] Inventors: Makoto Hayashi; Masanori Hinata; Minoru Yokota; Takasi Kondo, all of Osaka, Japan

[73] Assignee: Sumitomo Electric Industries, Ltd., Osaka, Japan

[22] Filed: Feb. 6, 1975

[21] Appl. No.: 547,853

|           |         |                     |          |
|-----------|---------|---------------------|----------|
| 3,178,925 | 4/1965  | Nolan et al. ....   | 72/467 X |
| 3,344,636 | 10/1967 | Pugh .....          | 72/271 X |
| 3,750,264 | 8/1973  | Nilsson .....       | 72/60 X  |
| 3,777,362 | 11/1973 | Nilsson et al. .... | 72/60 X  |
| 3,780,554 | 12/1973 | Nilsson .....       | 72/60    |
| 3,841,129 | 10/1974 | Nishihara.....      | 72/60    |

Primary Examiner—C. W. Lanham

Assistant Examiner—Joseph A. Walkowski

Attorney, Agent, or Firm—Sughrue, Rothwell, Mion, Zinn & Macpeak

[30] Foreign Application Priority Data

Feb. 6, 1974 Japan..... 49-15614

[52] U.S. Cl. .... 72/60; 72/56; 72/271; 72/467

[51] Int. Cl.<sup>2</sup> ..... B21C 23/22

[58] Field of Search ..... 72/56, 60, 271, 467

[56] References Cited

UNITED STATES PATENTS

2,218,459 10/1940 Singer ..... 72/467 X

[57]

## ABSTRACT

A hydrostatic extrusion process for producing relatively fine gauge wires less than  $250\mu$  in diameter, wherein a liquid providing a viscosity less than 100 poise at a pressure 10,000 atmospheric is employed as the pressure medium contained in the high pressure container.

2 Claims, 1 Drawing Figure





## HYDROSTATIC EXTRUSION PROCESS FOR PRODUCING FINE GAUGE WIRES

### BACKGROUND OF THE INVENTION

#### 1. Field of the Invention:

This invention relates to a hydrostatic extrusion process for producing wires, particularly extremely small gauge wires of copper, copper alloys, aluminum, aluminum alloys, gold, platinum, stainless steel and others less than  $250\mu$  in diameter.

#### 2. Description of the Prior Art:

In the prior art hydrostatic extrusion processes which are commonly used for producing metallic wires greater than 1 mm in diameter, a high viscosity liquid such as caster oil is favorably employed for the pressure fluid in order to reduce the friction on the die face. A relatively thick fluid lubrication film of the high viscosity liquid which is formed between the die face and the outer surface of the metallic wire being extruded through the die at a high speed is on the order of several microns and is thus sufficient to reduce the friction and provide an adequate fluid lubricated condition for the hydrostatic extruded wire.

In the production of relatively fine gauge metallic wires less than  $250\mu$  in diameter, however, such prior art technique developed for relatively large diameter wires can not fully achieve its intended objects and the wire is still subjected to a number of problems, such as the occurrence of break.

### SUMMARY OF THE INVENTION

It has been found by the inventors that particularly in the hydrostatic extrusion of wires with diameter less than  $250\mu$ , the effect of friction resistance of the pressure liquid acting on the surface of the wire is more important than the actual unfavorable effect of friction less action on the die surface, and that the hydrodynamic lubricated condition which is considered favorable for the hydrostatic extrusion of relatively large diameter wires tends to adversely affect the surface characteristics of the wire product less than  $250\mu$  in diameter.

The primary object of the invention is to provide a hydrostatic extrusion process which is particularly adapted for the production of fine gauge wires less than  $250\mu$  in diameter, and wherein such fine gauge wires can be produced easily and reliably at speeds higher than 200 m/min which is an important factor determining the commercial feasibility of the process.

It is another object of the invention to provide a hydrostatic extrusion process for producing metallic wires less than  $250\mu$  in diameter which utilizes a specific pressure fluid having a viscosity which is determined in relation to the conditions and characteristics of the hydrostatic wire stretching.

It is a still another object to provide a hydrostatic extrusion process for producing metallic wires less than  $250\mu$  in diameter which utilizes a specific die having an approach angle related to the condition and characteristics of the hydrostatic wire stretching.

It is a further object to provide a hydrostatic extrusion process for producing metallic wires less than  $250\mu$  in diameter which utilizes as the pressure fluid a slow viscosity liquid exhibiting a viscosity less than 100 poise under a pressure of 10,000 atmospheres.

It is a still further object to provide a hydrostatic extrusion process wherein fine gauge metallic wires less

than  $250\mu$  in diameter are extruded through a specific die having a die angle greater than  $35^\circ$  while using as the pressure fluid a low viscosity liquid exhibiting a viscosity less than 100 poise under a pressure of 10,000 atmospheres.

Additional objects other than those specifically stated will become apparent on consideration of the accompanying drawing and when considered in conjunction with the specification and claims.

### BRIEF EXPLANATION OF THE DRAWING:

The single FIGURE is a diagrammatic view showing the relationship between the pressure of liquid used as the pressure medium for hydrostatic extrusion and the frictional resistance imparted to the wire and wherein the notation is as follows:

- $\eta$ : A viscosity of pressure medium
- $V_2$ : wire velocity after passing through die
- $V_1$ : wire velocity before passing through die
- $R_2$ : extruded wire radius
- $R_1$ : supply wire radius
- $P_e$ : pressure of liquid
- $\tau$ : viscosity resistance
- $l$ : length of supply wire
- $h_0$ : spacing between inner wall of container 4 and supply wire 1
- T: tension

### DETAILED DESCRIPTION OF THE INVENTION

A preferred embodiment of the hydrostatic extrusion process in accordance with the invention will now be described in reference to the FIGURE.

A pressure medium 3 as well as the supply wire 1 is disposed within a pressure tight container 4 incorporating a die 2 located at the outlet end thereof through which the wire 1 is drawn and extruded outside the container 4.

The container 4 is placed in communication through a conduit 5 with a pump 6 for keeping the pressure medium 3 at the desired pressurized condition.

As the wire 1 is extruded through the die 2 at the rate  $V_2$  under tension T, a force or pressure component is provided by the friction between the wire 1 and the pressure fluid 3 which acts in the opposite direction to the movement of the billet, the magnitude of such force component being represented by the following approximation:

$$\frac{8 l \eta}{h_0 R_2 R^{3/2}} V_2 = P_e - P_i \quad (1)$$

where

- $\eta$ : viscosity
- $V_2$ : wire velocity after passing through die
- $R_2$ : wire radius after passing through die
- R: extrusion ratio
- $P_e$ : actual extrusion pressure
- $P_i$ : normal extrusion pressure
- $l$ : length of moving supply wire
- $h_0$ : spacing between container wall and supply wire (approximately half of internal diameter of container)

The pressure increase designated by  $(P_e - P_i)$  in the equation (1) is caused by viscous drag of the pressure medium and thus corresponds to tension or pulling force acting on the wire away from the die in a usual drawing process.

The magnitude of unfavorable effect of this pressure increase becomes greater with decrease of the extruded wire diameter and, in the case of producing wires less than  $250\mu$  in diameter, it often causes a break in the wire being extruded. This problem is particularly acute in the high speed hydrostatic extrusion of such fine gauge wires which requires a wire velocity after the wire passes through the die of over 200 m/min, preferably higher than 1,000 m/min.

The use of high viscosity liquid, such as castor oil, for the primary component of the pressure medium which has heretofore been employed for smoothing the hydrostatic extrusion process for relatively large diameter wires provides no means to prevent the above problem. On the contrary, it has been found that the pressure medium in the production of particularly fine gauge wires must be selected to have a relatively low viscosity ( $\eta$ ) satisfying the following relation:

$$\eta < \frac{1}{8} \frac{h_0}{v_2} \cdot \frac{l}{l} Y R_2 R^{3/2} \quad (1)$$

where

$Y$ : tensile strength of supply wire

$V_2$ : desired wire velocity after passing through die (greater than 200 M/min)

The other terms of the formula being identified in equation (1).

Among many liquid mediums providing such low viscosity, kerosine, gasoline, propanol, ethanol, ethylene-glycol and butanol are representative.

As will be understood by reading the examples hereinafter described, pressure fluid providing a viscosity less than 100 poise under a pressure of 10,000 atmospheres have proved satisfactory.

It has also been found by the inventors that the fluid lubrication characteristics which is effectively employed in hydrostatic extrusion processes for producing relatively large diameter wires results in a roughened wire surface which becomes increasingly appreciable as the thickness of the lubricant film increases, and does not achieve its intended effects in the case of hydrostatic extrusion process for fine gauge wires using a diamond die which effectively prevents sticking of metal.

The roughening of the wire surface by the thick fluid film lubrication characteristics may also be encountered in the high speed extrusion drawing processes which employ an extruded wire velocity on the order of 1,000 m/min and using a low viscosity pressure medium selected in the manner described above.

In order to eliminate this problem, the extrusion die should be selected to have a die semi-cone angle ( $\alpha$ ) which will prevent a fluid lubricated condition provided by the following approximate relation:

$$v_2 \geq \frac{Y}{\eta} \left[ \frac{6}{R \tan \alpha} \left\{ \frac{1}{2 \sqrt{R h t}} + \frac{\sqrt{R h t}}{h_1^2} - \frac{1}{h_1} \right\} + \frac{8l}{h_0 R_2 R^{3/2}} \right]^{-1} \quad (2)$$

In other terms, the die semi-cone angle ( $\alpha$ ) of the die must be selected to satisfy the following relation:

$$v_2 < \frac{Y}{\eta} \left[ \frac{6}{R \tan \alpha} \left\{ \frac{1}{2 \sqrt{R h t}} + \frac{\sqrt{R h t}}{h_1^2} - \frac{1}{h_1} \right\} + \frac{8l}{h_0 R_2 R^{3/2}} \right]^{-1} \quad (B)$$

where

$\alpha$ : semi-cone angle of die

$h t$ : difference between half of inner diameter of die and half of final diameter of extruded wire

$h_0$ : difference between half of maximum inner diameter at inlet of die and half of supply wire diameter.

The other terms in the formula being identified in formulas (1) and (A).

From the standpoint of commercial feasibility, it is desired in the extrusion of fine gauge wires to use a specific die having a die angle greater than  $35^\circ$  and constructed from diamond or other materials which do not readily stick to metals.

### EXAMPLE 1

15 A  $180\mu$  diameter supply wire of soft copper was drawn through a diamond die constructed to produce a finished wire product of  $100\mu$  diameter under a liquid pressure of  $500 \text{ kg/cm}^2$  lower than the pressure at which extrusion is started without exerting any pulling force to the wire.

This procedure was repeated on a number of samples while varying the type of pressure medium and the die angle. The maximum extruded wire velocities which permitted sufficiently long-time stability in the continuous extrusion operation under the varying condition, are shown in Table 1.

TABLE 1

| Pressure Medium      | Die Angle | Maximum Wire Speed (Extruded Wire Speed) |
|----------------------|-----------|------------------------------------------|
| Castor Oil           | 20°       | Less than 10 m/min                       |
| Methanol             | 30        | regardless of die angle                  |
| (4 : 1)              | 45        |                                          |
| Glycerin             | 20        | Approximately 100 m/min.                 |
| Ethylene-glycol      | 30        | Higher speed than this                   |
| (4 : 1)              | 45        | often result in wire break               |
| First Grade Lamp Oil | 20        | Up to the maximum                        |
| Kerosene             | 60        | take up speed (2,000 m/min)              |
| Gasoline             | 20        |                                          |
|                      | 30        | Same                                     |
|                      | 60        |                                          |

40 The test results of Table 1 indicate that low viscosity pressure medium such as kerosene or gasoline, etc., facilitates high speed extrusion for the production of fine gauge wires whereas when using a high viscosity pressure medium containing castor oil as the primary component which is favorably employed in the production of relatively large diameter wires, the extruded wire speed can not be increased sufficiently in the production of fine gauge wires.

45 It is noted that the viscosity of castor oil under the extrusion pressure (about 6,500 atmospheres) is 20,000 poise while the viscosity of glycerin under the same pressure is 100 poise, and kerosene and gasoline have lower viscosity than glycerin.

### EXAMPLE 2

Samples of soft copper wire  $45\mu$  in diameter were

extruded through a die having a die angle of  $45^\circ$  and

designed for an extruded wire product of  $25\mu$  diameter, under varying condition identical to that described in Example 1. The maximum permissible extruded wire speeds encountered in the individual tests are shown in Table 2. The test results of Table 2 demonstrate the favorable effect of using a low viscosity oil as the pressure medium still more clearly than do the test results of Table 1. In order to achieve a commercially feasible extrusion rate  $v_2$  higher than 200 m/min, it has been found necessary to use a low viscosity pressure medium such as kerosene or gasoline, etc.

TABLE 2

| Pressure Medium          | Maximum Extruded Wire Speed                                                            |
|--------------------------|----------------------------------------------------------------------------------------|
| Castor oil-Methanol      | Impossible to extrude at substantial speeds without causing break. (less than 1 m/min) |
| Glycerin-Ethylene Glycol | Less than 100 m/min for stable extrusion. Higher speeds caused break.                  |
| First Grade kerosene     | Up to 2,000 m/min, assuring stable extrusion at all times                              |
| Gasoline                 | Same                                                                                   |

## EXAMPLE 3

A supply wire of soft copper of  $80\mu$  diameter was extruded through a die having a die angle of  $60^\circ$  and designed to produce an extruded wire of  $40\mu$  diameter while using a pressure medium consisting of glycerin and ethylene glycol mixed in the ratio of 4 : 1. The temperature of the pressure medium was increased while the pressure thereof was maintained at 10,000 Kg/cm<sup>2</sup>. The maximum permissible extruded wire speeds determined at different temperatures are shown in Table 3. The test results confirm that a reduction in the viscosity of the pressure medium contributes to considerable increase in permissible extruded wire speed.

TABLE 3

| Temperature of Pressure Medium | Maximum Permissible Extruded Wire Speed                | Viscosity of Glycerin |
|--------------------------------|--------------------------------------------------------|-----------------------|
| 25°C                           | Less than 400 m/min                                    | 500 poise             |
| 70°C                           | Up to 2,000 m/min, assuring stable extrusion operation | 10 poise              |

## EXAMPLE 4

Samples of supply wire were extruded through dies having different die angles at various extruded wire speeds. The surface roughening was examined with respect to each of the samples after being extruded, the results being shown in Table 4. The test results of Table 4 confirm that die approach angles greater than  $35^\circ$  will effectively prevent the wire surface from becoming roughened or marred in the high speed hydrostatic extrusion drawing process using an extruded wire speed higher than 1,000 m/min.

TABLE 4

| Extruded Wire Speed<br>(m/min) | Die Angle |     |       |       |        |
|--------------------------------|-----------|-----|-------|-------|--------|
|                                |           | 500 | 1,000 | 1,500 | 20,000 |
| 5                              | 20°       | Δ   | X     | X     | X      |
|                                | 25°       | Δ   | X     | X     | X      |
|                                | 30°       | ○   | X     | X     | X      |
|                                | 35°       | ○   | ○     | Δ     | X      |
|                                | 40°       | ○   | ○     | ○     | Δ      |
|                                | 45°       | ○   | ○     | ○     | Δ      |
| 10                             | 60°       | ○   | ○     | ○     | ○      |
|                                | 90°       | ○   | ○     | ○     | ○      |

X: considerably roughened

Δ: partially roughened

○: non-roughened

15 While in the above examples kerosene, gasoline monomer and glycerin-ethylene glycol heated up to 70°C were employed by themselves as the pressure medium, these liquids may be used as a mixture thereof and may be heated sufficiently to provide a viscosity less than 100 poise at a pressure of 10,000 atmospheres. Further, a fatty acid, an extreme-pressure additive and the like may be added to the pressure medium to improve the wettability and lubrication property.

20 It should also be noted that the method of the present invention is applicable to wire production with any kind of metal, not just copper. For example, fine gauge wires of aluminum, gold, stainless steel and others can readily be produced in accordance with the method of the invention.

25 From the foregoing, it will be appreciated that the invention provides an improved hydrostatic extrusion method which employs a specific pressure medium providing a limited viscosity and a specific die having a limited die approach angle, and wherein relatively 30 small gauge metal wires less than  $250\mu$  in diameter can be produced with improved product quality and substantially cheaply as compared to the prior art extrusion drawing process.

35 What is claimed is:

1. In a hydrostatic extrusion process for producing relatively fine gauge wires less than  $250\mu$  in diameter by liquid pressure extruding a metal ingot of larger diameter than that of a die opening, through said die opening of a high pressure container, the improvement wherein a liquid providing a viscosity less than 100 poise at a pressure of 10,000 atmospheric is employed as the pressure medium contained in the high pressure container.
2. In a hydrostatic extrusion process for producing relatively fine gauge wires less than  $250\mu$  in diameter, by liquid pressure extruding of a metal ingot of larger diameter than that of a die opening, through said die opening of a high pressure container, the improvement wherein a liquid providing a viscosity less than 100 poise at a pressure of 10,000 atmospherics is employed as the pressure medium contained in the high pressure container and the wire is extruded through said die which has a die approach angle greater than  $35^\circ$ .